# EUROPEAN PATENT SPECIFICATION

(11) **EP 1 817 434 B1**
(45) Date of publication and mention of the grant of the patent: **17.11.2010**
(21) Application number: 04787621.4
(22) Date of filing: 30.09.2004
(51) Int. Cl.: C14C 1/00

(54) **CHEMICAL TREATMENT OF ANIMAL SKINS**
CHEMISCHE BEHANDLUNG VON TIERHÄUTEN
TRAITEMENT CHIMIQUE DES PEAUX D'ANIMAUX

(43) Date of publication of application: 15.08.2007
(73) Proprietor: Santori, Alberto, 63019 Sant'Elpidio a Mare (IT); Recanati, Giancarlo, 63019 Sant'Elpidio a Mare (IT)
(72) Inventor: SANTORI, Alberto, 63019 Sant'Elpidio a Mare (IT); RECANATI, Giancarlo, 63019 Sant'Elpidio a Mare (IT)
(74) Representative: Faggioni, Carlo Maria
(86) International application number: PCT/IT2004/000540
(87) International publication number: WO 2006/035468

(56) References cited:
- EP-A- 0 519 399
- DD-A5- 284 695
- DE-A1- 19 710 713
- GB-A- 834 403
- US-A- 3 426 557
- DATABASE WPI Section Ch, Week 198314 Derwent Publications Ltd., London, GB; Class A97, AN 1983-34059K XP002330371 & SU 931 744 B (LEATHER SHOE IND) 5 June 1982 (1982-06-05)
- DATABASE WPI Section Ch, Week 198612 Derwent Publications Ltd., London, GB; Class D18, AN 1986-079890 XP002330372 & RO 87 488 A (INTR ROMANA PIELE TIMISOARA) 30 August 1985 (1985-08-30)
- DATABASE WPI Section Ch, Week 198817 Derwent Publications Ltd., London, GB; Class D18, AN 1988-117485 XP002330373 & SU 1 337 413 A (LEATHER SHOE IND RE) 15 September 1987 (1987-09-15)

## Description

### FIELD OF THE INVENTION

The present invention refers to a tanning process, for tanning animal skins, which is particularly echological and environment friendly, and to an apparatus to carry out the process.

### BACKGROUND OF THE INVENTION

Tanning process is critical from the standpoint of environment. On one hand, tanning avoids the skin putrefaction, preventing the build up of CO2, which is dangerous for the greenhouse effect. On the other hand, the process usually employs a lot of substances, which are dangerous both for the worker health and for waters, where the outlet is drained.

Tanning process starts from a raw skin, which exhibits poor strength, which can be putrefacted and which shows unregular shape and leads to a final skin having good resiliency, high strength and which is stable with a constant thickness. Usually, the employed skins come from butcher's wastes.

Tanning process can be divided into three phases: a) from raw material to wet blue; b) from wet blue to crust; c) from crust to finished product.

The raw material should be selected so as to be as uniform as possible. The selected raw material is soaked with a mechanical treatment comprising dry drum tannage and a temperature increase, up to 28-30 °C, and a chemical treatment, including the addition of bases (e.g. NaOH, Na2CO3, NaHCO3, MgO), the addition of surfactants, antibacterials and protheolithic enzymes (catalysts).

Next step is lime-tip, in order to remove hair and epidermis, to obtain a good, fibrous collagen relaxation and a partial saponification of skin natural fat. In this step the skin is submitted to a treatment with a combination of lime, sulphide and sulphydrate, in the same drum tannages and reels used in the soaking. This step is the most polluting one. Table 1 reports the composition of the pollution.

**TABLE 1 - Main pollutants in lime-tip step**

| Pollutant | Concentration (mg/l) | Concentrations allowed |
|---|---|---|
| Sulphide | 2,000-5,000 | 1 |
| COD | 35,000-45,000 | 100 |
| BOD | 11,000-30,000 | 40 |
| Suspended particles | 25,000-40,000 | 80 |
| Total solids | 70,000-80,000 | 80 |
| pH | 11.0-12.5 | 5.5-9.5 |

Next step is lime removal. The lime deposited onto the surface of the skin is removed with a sufficient amount of water. Chemically bonded lime is removed through weak acids and through organic and inorganic acid salts. The latter sub-step leads pH to 8.3, which is the optimum value for enzymes to work. pH lowering should be as smooth as possible.
Bating is the following step. The use of enzymes removes remaining wastes and improve skin quality. Usually employed enzymes are pancreas enzymes, fungi enzymes and bacteric enzymes.
The skin is subsequently degreased, by adding surfactants and similar.
After degreasing, the skin is pikelled, by buffering strong acids with salts.
The so treated skin is then subjected to tanning. Three classes of tannants are used: polyaromatic tannants, mineral tannants and aliphatic tannants. Polyaromatic tannants can be divided into vegetable tannants and synthetic tannants. Vegetable tannants can be pyrogallol hydrolysed, like oak, chestnut, cherry plum, smoke-bush or valonea wood, and pyrocatechin condensates, like quebracho, mimosa, gambier. Synthetic tannants can be phenolic, like whole substitution tannants, or non-phenolic, like auxiliary and bleaching tannants. Usual mineral tannants are chrome, aluminium or zirconium tannants. Aliphatic tannants are aldehyde tannants, like formaldehyde, glutaric dialdehyde or amido dialdehyde, policondensation products, like methiol melamine, methiol dicyanamide or acrilates or paraffin derivatives, like sulpho chlorinated paraffines or fish oil.

Chrome tanning is by far the most popular tanning in the world. Chrome tanned wet blue are raw skins more and more diffused. A standard is at least 2% chrome, with a pH value between 3.5 and 4. The whole process needs from 48 to 96 hours. Therefore, it is apparent that a faster process, involving a smaller production of pollutants is strongly sought.

Another known process is described in WO 01/42514A. In such a process, a skin is treated after carrying it on a supporting plate which is introduced into a container, which is kept under vacuum during the introduction of a liquid mixture. Although such a process tries to perform as environment friendly, it is very complicate to carry out, very expensive and leads to very poor results.

EP-A-0 519 399 relates to a process for depilation of animal skins in which the skin is maintained in contact with an oxidising solution. After that a mechanical hair removal takes place. The oxidising solution is a foam. DD-A- 284 695 disclose a process for depilation of animal skins, according to which the skin is submitted to a solution of sodium hydroxide and hydrogen peroxide. SU 931 744 refers to a treatment of animal skin with hydrogen peroxide, polyvinyl alcohol and mineral salts. RO 87 488 refers to a process for treating animal skin with water, perhydrol and nitric acid. GB 834 403 discloses a method for treating a number of materials with a liquid under cavitation conditions, so as to cause ultrasonic irradiation, keeping the material rigidly supported and moving a series of liquid disturbing members. DE-A-19 710 713 discloses a device to detect the filling degree of a washing drum, which is able of rotation, the detection system comprising a ultra-sound source.

### SUMMARY OF THE INVENTION

The present invention refers to a tanning process for tanning animal skins, comprising a depilation step carried out through a pre-oxidation, wherein during such pre-oxidative depilation the skin is washed at 27°C in water, sodium carbonate (0.2 wt.%), hydrogen peroxide or ozonised water and thioglicolic acid, **characterised in that** said pre-oxidation step is carried out in the presence of ultra-sounds.

### BRIEF DESCRIPTION OF THE DRAWINGS

Fig. 1 is a side-view, partially in section, of a drum used for carrying out the process according to this invention; and
Fig. 2 shows a detail of Fig. 1.

### BEST WAY OF CARRYING OUT THE INVENTION

The inventive process for tanning animal skins involves a pre-oxidation step. All percentages reported in the following are by weight. Process conditions are to be calibrated on the particular skin to be tanned. The skin is washed at 27 °C in water, sodium carbonate (0.2%), ozonised water and thioglycolic acid, in order to make a complete dehaving and a partial dissolution of the back hidden fleshings. Preferably, sodium carbonate is 2.9-3.3%, ozonised water is 1 - 1.2% (giving 0.35 moles of O₂ per liter of solution and thioglycolic acid is 0.5%, the remainder (or hydrogen peroxide) being water. The solution is added in ca. 20 minutes, using a revolving drum 1. The revolving drum 1 used for the process according to this invention is represented in the drawings. It comprises two supports 2, which are integral with an internal core 3. Preferably, the said core 3 is cylindric. It accomodates a series 4 of ultra-sonic devices. About the core 3, some rotating blades 5 are provided. The drum 1 is connected to an ozone supplier, if ozonised water is the selected oxidating agent. The ozone supplier could be connected to a recycling water pipe, in order to remove the hair suspended in the water.

The diametre of the core 3 is chosen so that water, which should in any case equal the weight of the skin, in any case keeps the series 4 under its surface, so as not to shock ultra-sonic devices.

During the operation, the drum 1 is full of water and of the above solution. Preferably, ozone is bubbled in the water. The motion of the skin is performed by blades 5, which are connected to the core 3. Ultra-sonic devices are activated.

Subsequently, the treatment lasts for 7 hours with ultrasounds, at 23-25 °C. Ultrasound frequency is properly chosen depending on the skin thickness. Thereafter, temperature should never be over 28 °C. Oxidation agents other than ozonised water (or hydrogen peroxide) can be chosen, from the group consisting of fluorine, oxygen, ozone, nitric acid, sodium perborate and sulphuric acid. In any case, ozonised water is particularly preferred, since it gives no harmful waste.

Then, the pre-oxidated skin is treated with acids and possibly oxidised in acid environment.

As it can be easily be seen, no pollutant, or less pollutant than in conventional tanning processes is introduced. A comparison between pollutant in conventional processes and in the inventive one is reported in Table 2.

**Table 2 - comparison between conventional and inventive process**

| Pollutant | present lime-tip (mg/l) | inventive process (mg/l) |
|---|---|---|
| sulphyde | 2,000-5,000 | No |
| COD | 35,000-45,000 | 10,000-12,000 |
| suspended particles | 25,000-40,000 | 2,000 |
| total particles | 70,000-80,000 | 5,000-7,000 |
| chloride | 3 | no (with buffered acids) |

Since the inventive process does not involve toxic amounts of substances, the stripped fleshings can be used, in order to prepare fertilisers, animal food or similar. It is also possible to avoid the use of surfactants, like nonylphenols.

Preferably, non-toxic dyes are used to dye the tanned skin. Among them, food dyes, like anylines, are preferred as well as some vegetable extracts. Preferably, they are employed in an amount of 2-3 wt.%. The skin is rotated for 180 minutes in a revolving drum.

During each step of the inventive process, the temperature should be controlled, so as not to increase above 28-30 °C. An additional, optional step is to remove the hair by immunisation, without its destruction. In this way hair is in the flesh and it gives rise to no COD. In order to bate the skin, pH should be lowered up to 8-8.5. The oxidation step can be carried out both in acid, neutral and basic environment. Last step is tanning. Tanning is usually performed in two steps. First step is the so-called neutral tanning. It could be based either on silicates, or on caoutchouc, or on vegetables or on a combination thereof. The combination of vegetable and caoutchouc based tanning is preferred. It is preferably carried out in a bath containing H2O, 10% Tara extract and 4% caoutchou extract; the skin is rotated for 120 minutes in a revolving drum, up to a final pH of 3.8.

The secondo step is the so-called post tanning. After pressing and shaving skin, it is kept at a temperature of 45-47 °C. It is degreased with a natural extract, for instance a fish extract. The extract is preferably employed as 7-8 wt.% of the shaved skin.

Between the two steps of tanning, the skin is broken and shaved, so as to recover the shaving without environmental problems.

The skin obtained according to this invention exhibits features, which are new and never found in the market.

Summing up, the present invention provides a new tanned skin, through an environment friendly process, which allows even a time saving in the processing (up to 50%).

## Claims

1. A tanning process for tanning animal skin, comprising
a pre-oxidation, wherein during such pre-oxidation the skin is washed at 27 °C in water, sodium carbonate (0.2 wt.%), hydrogen peroxide or ozonised water and thioglicolic acid, **characterised in that** said pre-oxidation step is carried out subsequently in the presence of ultra-sounds for 7 hours at 23-25 °C.

2. A process as claimed in claim 1, **characterised in that** sodium carbonate is 2.9-3.3 wt.%, ozonised water is 1-1.2 wt.% and thioglycolic acid is 0.5 wt.%

3. A process as claimed in claims 1 or 2, **characterised in that** it further comprises the step of an acid treatment.

4. A process as claimed in claim 3, **characterised in that** it further comprises an acid oxidation step.

5. A process as claimed in any previous claim, **characterised in that** it includes a step of neutral-tanning.

6. a process as in claim 5, **characterised in that** such step of neutral-tanning is based on silicates, caoutchouc, vegetables or on a combination thereof.

7. A process as claimed in claim 6, **characterised in that** neutral-tanning step is based on a combination of vegetable tannants and caoutchouc.

8. A process as claimed in claim 7., **characterised in that** said neutral-tanning step is carried out with a bath containing H₂O, 10 wt.% Tara extract and 4 wt.% caoutchouc extract.

9. A process as claimed in any previous claim, **characterised in that** skin dyeing is carried out with a non-toxic dye.

10. A process as claimed in claim 9, **characterised in that** such dye is chosen among food dyes, like anilines.

11. A process as claimed in any previous claim, **characterised in that** during the bathing step pH is controlled at 8-8.5.

12. A process as claimed in any previous claim, **characterised in that**, between the steps of tanning the skin is broken and shaved, so as to recover the shaving without environmental problems.

## Patentansprüche

1. Gerbverfahren zum Gerben von Tierhaut, umfassend eine Voroxidation, wobei während der Voroxidation die Haut bei 27°C in Wasser, Natriumcarbonat (0,2 Gew.-%), Wasserstoffperoxid oder ozonisiertem Wasser und Thioglykolsäure gewaschen wird, **dadurch gekennzeichnet, dass** der Voroxidationsschritt anschließend in Gegenwart von Ultraschall für 7 Stunden bei 23-25°C durchgeführt wird.

2. Verfahren nach Anspruch 1, **dadurch gekennzeichnet, dass** Natriumcarbonat 2,9-3,3 Gew.-% ist, ozonisiertes Wasser 1-1,2 Gew.-% ist und Thioglykolsäure 0,5 Gew.-% ist.

3. Verfahren nach Anspruch 1 oder 2, **dadurch gekennzeichnet, dass** es weiter den Schritt einer Säurebehandlung umfasst.

4. Verfahren nach Anspruch 3, **dadurch gekennzeichnet, dass** es weiter einen Säureoxidationsschritt umfasst.

5. Verfahren nach einem vorangehenden Anspruch, **dadurch gekennzeichnet, dass** es einen Neutralgerbungsschritt einschließt.

6. Verfahren nach Anspruch 5, **dadurch gekennzeichnet, dass** der Neutralgerbungsschritt auf Silikaten, Kautschuk, Pflanzen oder auf einer Kombination davon beruht.

7. Verfahren nach Anspruch 6, **dadurch gekennzeichnet, dass** der Neutralgerbungsschritt auf einer Kombination von pflanzlichen Gerbstoffen und Kautschuk beruht.

8. Verfahren nach Anspruch 7, **dadurch gekennzeichnet, dass** der Neutralgerbungsschritt mit einem Bad durchgeführt wird, das H₂O, 10 Gew.-% Tara-Extrakt und 4 Gew.-% Kautschuk-Extrakt enthält.

9. Verfahren nach einem vorangehenden Anspruch, **dadurch gekennzeichnet, dass** Hautfärbung mit einem nicht-toxischen Farbstoff durchgeführt wird.

10. Verfahren nach Anspruch 9, **dadurch gekennzeichnet, dass** der Farbstoff unter Lebensmittelfarbstoffen wie Anilinen ausgewählt wird.

11. Verfahren nach einem vorangehenden Anspruch, **dadurch gekennzeichnet, dass** während des Badschrittes der pH auf 8-8,5 eingestellt wird.

12. Verfahren nach einem vorangehenden Anspruch, **dadurch gekennzeichnet, dass** zwischen den Gerbschritten die Haut gebrochen und gefalzt wird, so dass die Falzschnitzel ohne Umweltprobleme zurückgewonnen werden.

## Revendications

1. Procédé de tannage pour tanner des peaux d'animaux, comprenant une pré-oxydation, dans lequel au cours de cette pré-oxydation, la peau est lavée à 27 °C dans de l'eau, du carbonate de sodium (0,2 % en poids), du peroxyde d'hydrogène ou de l'eau ozonisée et de l'acide thioglycolique, **caractérisé en ce que** ladite étape de pré-oxydation est réalisée subséquemment en présence d'ultrasons pendant 7 heures à 23 à 25 °C.

2. Procédé selon la revendication 1, **caractérisé en ce que** le carbonate de sodium représente de 2,9 à 3,3 % en poids, l'eau ozonisée représente de 1 à 1,2 % en poids et l'acide thioglycolique représente 0,5 % en poids.

3. Procédé selon les revendications 1 ou 2, **caractérisé en ce qu'**il comprend en outre l'étape d'un traitement acide.

4. Procédé selon la revendication 3, **caractérisé en ce qu'**il comprend en outre une étape d'oxydation acide.

5. Procédé selon l'une quelconque des revendications précédentes, **caractérisé en ce qu'**il comprend une étape de tannage neutre.

6. Procédé selon la revendication 5, **caractérisé en ce qu'**une telle étape de tannage neutre est basée sur des silicates, du caoutchouc, des végétaux ou sur une combinaison de ceux-ci.

7. Procédé selon la revendication 6, **caractérisé en ce que** l'étape de tannage neutre est basée sur une combinaison de tannants végétaux et de caoutchouc.

8. Procédé selon la revendication 7, **caractérisé en ce que** ladite étape de tannage neutre est réalisée avec un bain contenant H₂O, 10 % en poids d'extrait de Tara et 4 % en poids d'extrait de caoutchouc.

9. Procédé selon l'une quelconque des revendications précédentes, **caractérisé en ce que** la teinture des peaux est réalisé avec un colorant non toxique.

10. Procédé selon la revendication 9, **caractérisé en ce qu'**un tel colorant est choisi parmi des colorants alimentaires, comme les anilines.

11. Procédé selon l'une quelconque des revendications précédentes, **caractérisé en ce que** durant l'étape de bain, le pH est réglé de 8 à 8,5.

12. Procédé selon l'une quelconque des revendications précédentes, **caractérisé en ce que**, entre les étapes de tannage, la peau est cassée et rasée, de manière à récupérer le produit du rasage sans problèmes environnementaux.
